

# UNITED STATES PATENT OFFICE.

JOHN R. HYER, OF HERKIMER, NEW YORK.

## WATERPROOFING COMPOSITION.

1,405,220.

Specification of Letters Patent. Patented Jan. 31, 1922.

No Drawing.

Application filed June 28, 1921. Serial No. 481,073.

To all whom it may concern:

Be it known that I, JOHN R. HYER, a citizen of the United States, residing at Herkimer, in the county of Herkimer and State 5 of New York, have invented certain new and useful Improvements in Waterproofing Compositions, of which the following is a specification.

This invention relates to water-proofing 10 fabrics and while having especial reference to paper is applicable to fabrics other than paper with perhaps equal or greater benefits.

A further object of the invention is to provide a water-proofing and a fabric water- 15 proofed thereby which is thoroughly pliable and which presents no fracture of the water-proofing resulting from the bending of the fabric thus water-proofed.

A further object of the invention is to provide 20 means whereby paraffine and rosin, both well known water-proofing materials, may be applied to a fabric to provide a successful and satisfactory water-proofing and water- proofed fabric.

25 A further object of the invention is to mix with paraffine and rosin at a temperature sufficient to maintain liquidity Epsom salts which produces ebullition and thereby enables the fabric immersed therein to become 30 coated and partially impregnated with the material which is otherwise too heavy for manipulation.

It is probable that the ingredients above referred to may be employed in proportions 35 varying within certain ranges, but I have found that a mixture of 43% paraffine, 55% of rosin, and 2% of Epsom salts, by weight, produces an ideal compound for the purpose and that when maintained in liquid condition 40 by heat and paper, or other fabric, immersed therein, provides an ideal water-proofing and an ideal water-proofed fabric.

In the actual carrying out of the process the material is maintained in liquid condition 45 by heat in any convenient vat or recep-

tacle, and the paper, or other fabric immersed therein in any approved manner, as simply being drawn through the bath and the superfluous material adhering to the fabric preferably scraped off or removed by rollers, or 50 any usual and ordinary form of scraper, or the like, it being wholly immaterial in what manner the superfluous material is removed.

What I claim is:

1. A water-proofing composition comprising paraffine, rosin and Epsom salts. 55

2. A water-proofing coating composition comprising paraffine, rosin and Epsom salts commingled and maintained in liquid condition by heat. 60

3. A water-proofing composition comprising approximately 43% of paraffine, 55% of rosin and 2% of Epsom salts, by weight. 65

4. A water-proofed fabric comprising a sheet of material having adhering to its exterior a composition of paraffine, rosin and Epsom salts. 70

5. A water-proofed fabric having adhering to its exterior and impregnating its interstices a composition of paraffine, rosin and 75 Epsom salts.

6. A water-proofed fabric comprising a sheet of material having adhering to its exterior a composition of approximately 43%, 75% paraffine, 55% rosin and 2% Epsom salts. 80

7. A water-proofed fabric comprising a sheet of material having its interstices filled with a composition of paraffine, rosin and Epsom salts. 85

8. A water-proofing material comprising 80 a wax, a gum and a salt of magnesia.

9. A water-proofing composition comprising a mineral wax, a resinous material and a salt of magnesia.

In testimony whereof I hereunto affix my 85 signature in presence of two witnesses.

JOHN R. HYER.

Witnesses:

J. H. SHAILER,

FRANKLIN H. HOUGH.